

# UNITED STATES PATENT OFFICE.

FRANK E. JACOBS, OF WASHINGTON, DISTRICT OF COLUMBIA.

## SMOKE-PREVENTING COMPOUND.

No. 802,734.

Specification of Letters Patent.

Patented Nov. 3, 1903.

Application filed July 15, 1907. Serial No. 382,882.

*To fill whom it may concern:*

Be it known that I, FRANK E. JACOBS, a citizen of the United States, residing at Washington, in the District of Columbia, have invented a new and useful Smoke-Preventing Compound; and I do hereby declare the following to be a full, clear, and exact description of the invention, such as will enable others skilled in the art to which it appertains to make and use the same.

This invention relates to improvements in smoke preventing means and particularly to chemical compounds for securing a more perfect combustion of fuels.

The invention comprises means for enabling the wider use of the so-called bituminous or soft coals and similar fuels without the generation of large quantities of smoke.

One of the objects of the invention is to secure the full heating value of fuels economically.

Another object of the invention is to secure the full heating value of fuels without necessitating elaborate changes or additions to existing furnaces.

Another object of this invention is to prevent the production of smoke in the combustion of fuels, more especially the combustion of coals.

With these and other objects in view this invention comprises certain novel and useful combinations of parts, as will be hereinafter described and claimed.

If the process of combustion of coals, particularly of the so-called soft or bituminous coals, large volumes of unconsumed and uncombined carboniferous matter escape in the form of smoke, and permeate the surrounding atmosphere to the injury of health, comfort and vegetation. The explanation why different fuels give off different amounts of unconsumed substance or smoke is clearly seen in the chemical analysis of the various fuels. It is well known that anthracite or hard coal will generate less smoke than bituminous or soft coal, and that coke and charcoal will generate still less smoke than anthracite coal. The primary reason lies in the fact that anthracite coal possesses from 3 to 9 percent. of volatile matter of hydrocarbons, and from 73 to 87 per cent. of fixed carbons; while bituminous coal possesses from 19 to 41 per cent. of volatile matter or hydrocarbons and from 46 to 73 per cent. of fixed carbons.

On the other hand charcoal and coke are composed principally of ash

and carbon, with the latter greatly in predominance. The volatile or hydrocarbon matter of fuels consists in various compounds that are released from the fixed carbons during the process of combustion and form the basis of a large number of compounds, secured from coals by destructive distillation, possessing great calorific value, among which are the following direct products:—coal gas, of varying formula; ammonium ( $\text{NH}_4$ ), and compounds thereof; benzene ( $\text{C}_6\text{H}_6$ ); toluol ( $\text{C}_7\text{H}_8$ ); xylol ( $\text{C}_8\text{H}_{10}$ ); pyridin ( $\text{C}_5\text{H}_5\text{N}$ ); carbolic acid ( $\text{CO}_2$ ); naphthalene ( $\text{C}_{10}\text{H}_8$ ); pyrene ( $\text{C}_{10}\text{H}_{12}$ ); and anthracene ( $\text{C}_{14}\text{H}_{10}$ ); etc.

The process of coal combustion is divided into two phases: The first phase is marked by the volatilization and combustion of the hydrocarbons and varies with conditions; the second is marked by the combustion of the remaining carbon. The formation of smoke occurs during the volatilization of the hydrocarbons and varies with the supply of oxygen, the local temperature, and the amount of escaping hydrogen unconsumed. It has been determined by scientific investigation that a compound gas when sufficiently heated separates into its elements, and a sudden cooling of the heated gas will give a simple mixture instead of the original combination; a slow cooling reproduces the original gas. It has also been determined scientifically that new compounds are formed on heating the hydrocarbons to high temperatures, a part of the carbon being deposited as soot. These two phenomena undoubtedly go together in smoke production. It is recognized by those familiar with the nature of fuels that the phenomena of combustion cannot be sufficiently explained by present organic chemistry or physics. This is especially true in relation to the analysis of fuels to determine their coking qualities.

Since a unit of carbon affords about 8,000 calories of heat, while a unit of hydrogen affords 34,000 calories, it will be seen that hard coals, low in hydrogenous matters, must surrender an increased volume of fixed carbons to compensate for this difference, and therefore, bituminous coal appears to be the ideal fuel.

The problem of securing a more perfect combustion of fuels and to secure the elimination of smoke is both a mechanical and a chemical one. Certain conditions concerning the grates, drafts, etc. must be observed in any case, but the effort to solve the prob-

lem by a modification of these elements has been expensive and not always practical.

The object of the present invention is to provide a simple, chemical, solution without necessitating elaborate mechanical improvements in furnaces and appliances therefor.

This invention is the result of extensive experience and experimenting and its efficiency is confirmed by repeated trials and practical 10 demonstrations. It consists in a preparation of chlorid of sodium, (NaCl,) 1 lb.; carbonate of potassium, as a lye of potash, (K<sub>2</sub>CO<sub>3</sub>), 4 ozs.; oxalic acid, (C<sub>2</sub>H<sub>2</sub>O<sub>4</sub>) 4 ozs.; borax, (Na<sub>2</sub>B<sub>4</sub>O<sub>7</sub>, 10H<sub>2</sub>O,) 1 oz. These 15 ingredients are mixed together with ash, in the above proportions, in any quantity desired, and then mixed with the coal or fuel. The result is that a more perfect combustion of the coal, thus treated, is secured and the 20 formation of smoke is prevented.

The ingredients are preferably used in the commercial state, and they are, as is well known, charged with various impurities. It has been found for instance that ordinary 25 commercial potash, known under various names as potashes, potassa, pearlash, sub-carbonate of potassa, carbonate of potassium, and in solution with water as lye of potash, showed on analysis the following re- 30 sults:—

|                                                          | 1.    | 2.   | 3.    | 4.   |
|----------------------------------------------------------|-------|------|-------|------|
| Potassium carbonate K <sub>2</sub> CO <sub>3</sub> ..... | 74.10 | 62.6 | 68.07 | 41.7 |
| Potassium hydrate KOH.....                               |       |      |       | 49.6 |
| Sodium carbonate Na <sub>2</sub> CO <sub>3</sub> .....   | 8.0   | 11.0 | 5.85  | 1.4  |
| Potassium sulfate K <sub>2</sub> SO <sub>4</sub> .....   | 13.47 | 15.5 | 15.32 | 4.0  |
| Potassium chlorid KCl.....                               | 0.95  | 4.0  | 8.15  | 2.0  |
| Water H <sub>2</sub> O.....                              | 7.28  |      |       |      |
| Insoluble matter (?).....                                | 1.28  | 6.9  | 2.64  | 1.2  |

The analysis of a sample of anthracite ash 40 gave the following result:

|                         |             |
|-------------------------|-------------|
| Silica.....             | 53.60       |
| Alumina.....            | 36.69       |
| Sesquioxid of iron..... | 5.59        |
| Lime.....               | 1.08        |
| Oxid of magnesia.....   | 1.19 100.00 |

Coal ash has also been found to contain phosphorus, sulfur, and other elements.

In the present state of chemical knowledge 50 it is quite impossible to describe the chemical reactions that occur during the various stages of combustion of a coal or fuel treated with the above described compound. Since the chemical products of combustion, in part, 55 must be carbon dioxid and hydrogen oxid or water, and the physical state of the elements combined in coal is not understood, it is beyond the limits of our knowledge to approximate all the causes which result in the elimination of smoke by treating coal with this invention. Existing knowledge of hydrogen is based largely upon its actions as a gas, little is known of it as a solid hydrocarbon, and consequently little is known of the proximate 65 composition of coal, which is not a mere mix-

ture of hydrogen and carbon. The calorific value of the different hydrocarbons varies with their constitution, and that of solid carbon with its physical state, therefore, it is not easy at present to trace the relation between the results yielded by any given coal on analysis and those found in practical use. We do not know, therefore, what coal is proximately composed of—in what way the elements are combined in the substance—or what is the calorific value of its various ingredients or of the compounds which may be produced by treating it at different temperatures.

Among the requisites of perfect combustion are (1) intimate mixture and contact between the particles of the combustibles and the air, and not a mere access to a limited supply of air. (2) The maintenance of a suitable temperature for the chemical combination during the period of the combustion.

It is possible that the invention brings about a more perfect combustion of the coals or fuel, and the prevention of the formation of smoke, by peculiarly satisfying the above 90 conditions, and that it does this either by maintaining a proper average of temperature; by effecting a more intimate contact of the oxygen and the carbons and hydrogen; by decreasing the volatilizing tendency of 95 the hydrocarbons; by forming a partial inclosing barrier or coating upon the surface of the coals, and thus limiting the play of the oxygen, so that its energy may be given to the hydrocarbons first; or by establishing 100 new physical relations between the molecules of the coal during the process of combustion; or by satisfying a third unknown condition. But whatever the manner of operation or the exact influence of the invention on the combustion of coal may be, it does eliminate the 105 depositing of ungasified carbon and does increase the amount of heat generated. It is apparent, therefore, that the following elements are present during the combustion of 110 coal or fuel treated with the compound, which treatment may vary with the character of the coal or fuel, and other conditions. O, H, C, K, Cl, Na, Ca, Si, Mg, Fe, Al, B, P, S, and N.

It has been found that the proportions of the ingredients should be those given, though in practice the quantity of each ingredient may be slightly varied without departing from the spirit of my invention. The best 120 results, when using a good quality of bituminous coal, are secured by using the compound in the proportions specified.

I claim:

1. In combination, means for preventing 125 the formation of smoke during the process of the combustion of fuels, consisting in a mixture of oxalic acid, carbonate of potassium of commerce, borax, common salt, coal ash and sufficient water.

2. In combination, means for preventing the formation of smoke during the process of the combustion of fuels, consisting in a mixture of oxalic acid, a lye of carbonate of potassium of commerce, chlorid of sodium, and ash.

3. In a compound of the class described, a mixture of one pound of chlorid of sodium ( $NaCl$ ), four ounces of carbonate of potassium of commerce ( $K_2CO_3$ ), four ounces of oxalic acid ( $C_2H_2O_4$ ), one ounce of borax ( $Na_2B_4O_7 \cdot 10H_2O$ ) and ash.

4. A process for improving the heating qualities of fuels and preventing the same

from smoking during the process of their combustion, consisting in treating the fuel 15 with a mixture of oxalic acid, a lye of commercial carbonate of potassium, borax, chlorid of sodium, and ash.

In testimony whereof I have signed my name to this specification in the presence of 20 two subscribing witnesses.

FRANK E. JACOBS.

Witnesses.

H. L. FRANC,  
ANNA T. BURNS.